

Sept. 27, 1927.

1,643,400

J. A. WILSON

UPHOLSTERY PANEL AND METHOD OF MAKING THE SAME

Filed Feb. 17, 1921

Fig. 1



Fig. 2



4

2

Fig. 3



INVENTOR

John A Wilson

BY

Chester W. Bassett

ATTORNEY

Patented Sept. 27, 1927.

1,643,400

# UNITED STATES PATENT OFFICE.

JOHN A. WILSON, OF ELIZABETH, NEW JERSEY, ASSIGNOR TO DURATEX CORPORATION, OF NEWARK, NEW JERSEY, A CORPORATION OF NEW JERSEY.

## UPHOLSTERY PANEL AND METHOD OF MAKING THE SAME.

Application filed February 17, 1921. Serial No. 445,869.

This invention relates to improvements in upholsterty panels and the method of making the same and relates more particularly to such panels suitable for use in automobile bodies.

One object of the invention is to produce an upholsterty panel which simulates leather, yet which will be much cheaper than leather and easier of application.

Another object is to provide an improved method or process of making a coated article, preferably coated with a composition containing nitrocellulose, and embossed to simulate leather and which is suitable for use as a kick pad or door panel in an automobile.

Heretofore, that type of upholsterty panels were made of leather or artificial leather and usually consisted of a base of paper or cardboard upon which leather or leather substitutes has been rigidly secured by glue or other means with the edges of the leather or other substitute turned over the edges of the carrier board and fastened in place. Such panels, while possibly satisfactory, have entailed considerable labor and expense and one of the objects of this invention is to lessen the labor in producing upholsterty panels and cheapen the cost of their manufacture.

Further objects of the invention will definitely appear from the following detailed description and drawing showing a piece of fabric or panel in which:

Fig. 1 is a view of the waterproofed side of the panel.

Fig. 2 is a view of the embossed side of the panel.

Fig. 3 is a section through the panel in exaggerated detail showing the coating material, the basis and edges of the panel or fabric.

In general the objects of the invention are carried out by providing a suitable paper or pulp base with a coating of a composition containing nitrocellulose and embossing the same.

The pulp or paper used is preferably made waterproof as by varnish or similar material. The waterproof quality may either be provided at the time that the paper is manufactured or may be applied before the coating of composition is spread on the same.

Similarly where the article is to be used as a lining or door panel for an automobile or as a kick pad on such a vehicle, the paper may

either be cut to proper size and shape before the composition is applied to the same or, if desired, the composition and embossing may be spread upon the paper before cutting.

It is obvious that the mixture or composition used for coating this paper must be of such a nature that the film coating will not peal and therefore it has been found desirable to use some sort of substance as a gum or resin supplying an adhesive characteristic in conjunction with the nitrocellulose coating. Furthermore, the final solution used must also comprise some solvent that will dissolve not only the nitrocellulose, but also the gum or resin whichever is added or has been added to the composition. For this purpose, ethyl, butyl or amyl acetate is preferably employed, although any other suitable ester or an alcohol or other solvent having the properties above set forth may be employed. It has been found that in place of gum or resin, a bitumen may be used in conjunction with a nitrocellulose composition.

A preferred example of one formula, used with considerable success in practicing this invention, comprises one part by weight of shellac dissolved in a proper solvent, two parts of nitrocellulose dissolved in a required solvent, with the necessary amount of the desired shade of pigment, the latter being added either in dry form or ground with a vegetable oil.

The nitrocellulose composition outlined above is spread upon the paper or pulp base in any desired manner, either by hand or by machine, by means of a knife or brush, either by the use of rollers or by the use of a usual form of spreading knife, it may even be sprayed on, the sole requirement being that the coating be evenly and uniformly applied over the whole surface as indicated at 1, in Figs. 2 and 3. After spreading and drying the article is embossed either by plates or rollers usually employed in the manufacture of artificial or substitute leather as indicated at 2 in Fig. 2.

The coating is preferably of such slight thickness that the impressions of the embossing dies is carried through the nitrocellulose coating on to the very surface of the fiber board beneath as indicated at 3, in Fig. 3.

As the spreading of the coating as described above usually results in the setting up of a tension on the face of the cardboard or

paper used, it has been found desirable to size the opposite or uncoated side of the material with a suitable sizing or glue 4 and thus set up an equal tension on both faces 5 of the cardboard or paper. It has been found that such sizing of the reverse side of the article successively prevents any warping or bending of the panel.

The finished product is now left to thoroughly dry, usually by the application of 10 heat and air to permit the solvents used during the process to completely evaporate.

As the finished article is to be used in a substantially vertical position and subject 15 more or less to the elements, it becomes necessary to protect the cut edges not only around the outer periphery of the panel but also that of the hole for the pocket, for instance. To this end therefore, these cut edges are water- 20 proofed, preferably by the composition containing the nitrocellulose and therefore the preferred practice is to first cut the paper or cardboard base of proper size and configuration and provide it with the necessary open- 25 ings for the door handle and pocket, in case of a door panel, and then coat with composition which is to carry the embossing.

The coated article made as described is particularly suitable for upholstery purposes 30 as set forth in connection with the inner door lining of an automobile door or as a kick pad, that is the vertical front face of an automobile seat. The new product is much 35 cheaper to make and at the same time is fully as durable as a panel in which the artificial or substitute leather is first spread on a fabric or thin paper carrier and then glued to the cardboard.

Believing that the above-described process 40 and product, using nitrocellulose, are new, it is desired to claim the same broadly, without reference to the particular ingredients used in connection as colors and as adhesives, other than nitrocellulose as used in the coating 45 composition.

Being aware that the particular embodiment of the invention shown and described

is susceptible of considerable variation without departing from the spirit of the invention, therefore, it is desired to claim the same 50 broadly as well as specifically, as indicated by the appended claims.

What is claimed is:

1. As a new article of manufacture, an upholstering panel comprising a fiber board coated with a composition comprising one part by weight of shellac, two parts by weight of nitrocellulose and containing the necessary amount of the desired shade of pigment. 55

2. An upholstered panel comprising a water-proofed fibre base having its face and edges coated with a composition of nitrocellulose and a shellac-like material, and having its uncoated side sized. 60

3. As a new article of manufacture, an upholstering panel comprising a fiber board one side and the cut edges of which are coated with a composition comprising one part by weight of a shellac-like material and two parts by weight of nitrocellulose. 65

4. The method of producing upholstery panels which comprises waterproofing a suitable fiber base, applying a thin uniform coating of composition containing nitrocellulose to one side of the same, embossing the latter side so that the configuration of the embossing extends into the surface of the fiber base, and drying the same. 70

5. The method of producing upholstery panels which comprises cutting a suitable fiber base of proper size and configuration, waterproofing one side and the cut edges of the base, applying composition containing nitrocellulose to the other side, then embossing the latter side, and drying the panel. 75 80

6. An article of the class described comprising a base material; a coating of waterproofing on one side and on the edges of the base material; and a coating of nitrocellulose composition on the other side of the base material. 85 90

In testimony whereof, I affix my signature.

JOHN A. WILSON.